

## UNITED STATES PATENT OFFICE

2,573,883

METAL COATING PROCESS AND OIL FINISH-  
ING COMPOSITION THEREFOR

George W. Waters, Wood River, Ill., assignor to  
Shell Development Company, San Francisco,  
Calif., a corporation of Delaware

No Drawing. Application April 12, 1947,  
Serial No. 741,002

17 Claims. (Cl. 117—51)

1

This invention relates to metal coating or alloying of metals. More particularly this invention pertains to oil compositions used in tinning, terne coating, lead coating, and the like, in order to facilitate and aid in coating or alloying a base metal with a uniform and tenacious metal coating.

This process, for example, the tinning process comprises essentially coating base metals by dipping and the like said metals into a bath of molten tin thereby coating the base metal with a thin film of metallic tin. The tinning process is carried out at elevated temperatures and when skillfully done with the aid of good fluxing agents and proper tinning oils actually forms an alloy of tin and the metal being treated which is generally iron, steel and other ferrous metals.

To insure strong adherence of the tin to the metal surface being coated, the metal must be absolutely clean and free of any grease, dirt, oxide film and rust. This is necessary to insure intimate contact of the metal with the molten tin, terne composition and the like. Metals which are to be coated with tin and the like are therefore carefully prepared by being properly mechanically and chemically treated, pickled and kept in slightly acidic solution in order to prevent oxidation of the metal surface prior to entering the tinning bath or the like.

Briefly stated, for example, one method of tin coating of base metals comprises dipping or passing a properly cleaned metal into a bath of molten tin, on to an oil bath and then through cleaners to remove excess oil and polish the tinned metal surface. The general procedure is to pass a mildly pickled metal plate from a slightly acidified storage tank into a tin pot usually divided into a series of compartments. Each compartment contains a series of rollers through which the metal can pass during its various stages of tin coating. The molten tin occupies the lower or bottom part of the tin pot. On the feed end of the pot floats a layer of flux and on the exit end floats a much deeper layer of oil.

The flux serves to give final preparation of the metal surface before being immersed into the molten tin. It consists generally of zinc chloride or mixtures of zinc chloride and sodium chloride or ferric chloride or ammonium chloride and the like. The function or purpose of the flux is to clean thoroughly the metal surface, remove moisture, absorb any oxide film, pickling scum and control more or less the wettability of the metal by the tin so that the mol-

ten tin would react and adhere uniformly and tenaciously to the metal surface treated.

From the fluxing bath the metal proceeds on through a series of rollers through a molten tin bath kept at a temperature of between about 525° F. to above about 750° F. depending upon the operating conditions. The tinned metal then proceeds through an oil bath while passing through rollers where excess tin is removed, better distribution of the tin coating is secured and oxidation of the tin is inhibited. The tinned metal having a thin film of oil on it proceeds on out of the oil bath and receives a cleaning treatment where excess oil is removed. Any remaining oil left on the metal aids in polishing the metal to a desired surface finish.

Articles of odd shape can be tin coated by mechanical or hand dipping into a flux coated tin pot and then redipped into an oil coated tin pot which on withdrawal comes in contact with the oil and receives its beneficial treatment. If desired the metal can then be immersed into a hot oil bath for final oil treatment in order to more closely control the thickness of the tin coating and also such oil treatments act to some degree as a quenching medium.

Tinning oils play a vital role in the tinplating art for they serve to secure better distribution of tin on the base metal being coated, aid in removal of excess tin and protect the tin from oxidation or discoloration while being cooled. To accomplish these and other features a good tinning oil must be capable of adsorbing oxides so as to keep the metal surface clean; it must have a suitable interfacial tension with molten tin and with the atmosphere and it must be stable and not tend to deteriorate or polymerize even after long periods of use under extremely high temperatures. Efficient tinning oils should in addition form a uniform film on the coated metal surface while in the tin pot but on immersing from the pot drain off easily and quickly. Oils which do not drain off easily must be continuously replaced which is quite an expense. Such oils also tend to form globules or isolated patches on the tinned surface which produce depressions on the tin coating, resulting in localities which are very thin and which form grease marks on the tinned surface.

One main criterion of a good tinning oil as stated above is its ability to drain off rapidly from the tinned article as it emerges from the hot oil bath. From this aspect straight mineral oils and even palm oil after relatively short periods of use are not satisfactory. This desirable phe-

nomenon of rapid draining seems to be associated with the presence of certain polar bodies in the oil. An oil containing a plurality of these polar bodies drains off rapidly and leaves the tinned surfaces clean and bright. It is assumed that such oil films tend to form one or more aggregates which move continuously over the surface in an apparently random fashion. As the activity of the aggregates becomes reduced owing to reduction of these polar bodies, the draining rate of the oil is reduced and eventually a "continuous film" state is reached where the draining properties of oils are considerably retarded and the oil is no longer suitable for use. It is postulated that the efficiency of such oils is due to the formation of a monomolecular absorbed layer over the surface of the tin.

Generally oils used in tinplating are subjected to elevate temperatures of at least 460° F. and higher for long intervals. It is therefore essential that such oils be chemically stable at such temperature, without undue volatilization, decomposition or polymerization.

Palm oil is known to be an efficient tinning oil. However, it has several serious drawbacks in that it is costly, difficult to obtain and above all polymerizes readily at temperatures above 470° F. resulting in sludging and high oil losses. Also other beneficial tinplate properties of palm oil are destroyed at temperatures above 470° F. At this elevated temperature palm oils leave on the tinplate streaks of oil resulting in a dull, lustreless coated surface. Other known tinning oils such as hydrogenated cottonseed oil present even more difficult tinning oil problems than palm oil and generally not as efficient.

It is an object of this invention to produce an excellent tinning oil having a petroleum hydrocarbon base. Another object of this invention is to produce a new and improved tinning oil which is stable at extremely high temperatures for long periods of time. Another object of this invention is to produce a new and improved tinning oil having the ability to take up oxide, to readily absorb flux residue and to promote the spreading of tin and other molten metals. Still another object of this invention is to produce a tinning oil which does not stain or have bad effects on the coated surface if left on. Furthermore, it is another object of this invention to produce a tinning oil which drains and cleans easily and which is not a fire hazard.

The above and other objects may be attained in accordance with the present invention by admixing with a mineral oil base a suitable amount of partially hydrogenated high molecular weight fish and/or marine oil distillates. The amount of partially hydrogenated high molecular weight fish and/or marine oil distillates which can be added to a mineral oil base should be sufficient to maintain the acid number of the tinning oil composition at not less than 3 and not above about 15, and preferably between about 4 to 10. In order to maintain the acid number of the composition at these values, a replenishing agent can be added to the oil at determined intervals. The replenishing agent comprises a concentrate of approximately equal parts by weight of mineral oil and hydrogenated fish and/or marine oil distillates and is added in amounts sufficient to adjust the acid number of the base composition to not less than 3 and not above about 15.

The partially hydrogenated fish and/or marine oil distillates and their mixtures can be obtained from codfish oil, codliver oil, dogfish oil, dolphin

body oil, dolphin fish oil, herring oil, Jap fish oil, menhaden oil, porpoise body and jaw oils, salmon oil, sardine and sardine liver oils, seal oils, shark and shark liver oils, sperm whale body and head oils, whale oil and the like.

The fish and/or marine oil distillate products of this invention, can be removed from such oils by a conventional means and then hydrogenated or the oils can be hydrogenated first and the product then split and the overhead distillate fraction removed by distillation, extraction and the like. For example a fish oil such as herring oil, menhaden oil and the like, can be hydrogenated and split and subsequently distilled to produce an overhead distillate of hydrogenated fish oil. The residue product is generally referred to in the trade as fatty acid residuum products or fish oil stearine pitches. The pitch can be further split, subjected to distillation, the overhead distillation fraction recovered, hydrogenated and combined with the first overhead distillate product and used as additive products in this invention. Another method of producing the desired distillate fractions is to split the oil first, remove the distillate fraction and then hydrogenate it preferably in the presence of a suitable catalyst and at elevated temperatures.

The overhead distillate product obtained from fish and/or marine oils and their mixtures which are used as the additives for tinning oils of this invention are not to be confused with the residue product generally referred to as stearine pitches or residuum products. The two materials are entirely separate and distinct and the stearine pitches are not contemplated for use in this invention since test results indicate, as will be hereinafter shown, that they are inferior to the distillate fractions as tinning oil additives.

|                      | Distillate | Residue |
|----------------------|------------|---------|
| Sp.gr., 60° F.       | 0.950      | 0.895   |
| M. P., °F.           | 145        | 134     |
| S. U. Visc., 210° F. | 47         | 49      |
| Sap. No.             | 190        | 199     |
| Acid No.             | 188        | 149     |
| Iodine No.           | 3.6        | 23      |

The mineral oil base used can be any suitable refined petroleum hydrocarbon stock having high flash and fire points and which are substantially stable at tinning temperatures of between about 460-490° F. Suitable petroleum hydrocarbon base stocks which can be used are solvent extracted Mid-Continent Bright stock, acid treated Mid-Continent Bright stock, acid treated naphthenic neutral stock and blends of these oil stocks. Preferably however solvent extracted Mid-Continent Bright stock having a Saybolt Universal viscosity at 210° F. of 150-170 is used as the oil base stock because of the superior tinplating results obtained when using this type of oil.

To more fully and clearly illustrate this invention a series of identical and parallel comparative tinning tests were conducted in which the tinning performance as to flux removal, drainage characteristic, ease of cleaning and spreadability characteristics of mineral oil, palm oil, mixture of palm oil and mineral oil, a composition comprising a mixture of mineral oil and hydrogenated fish oil residuum or stearine pitches and a mixture of mineral oil with hydrogenated fish and/or marine oil distillate products were compared.

One test was conducted as follows:

A. Pickled sheets of black plate, stored in 0.5

per cent HCl, were dipped in flux (3 pounds ZnCl<sub>2</sub> plus 5 ounces NH<sub>4</sub>Cl per gallon) and tinned at temperatures between about 530-560° F., and preferably at 550° F. The tinning pot surface was covered with flux. Sheets were tinned so that very little, if any, flux adhered to the sheets upon withdrawal. Immediately after withdrawal, the sheets were transferred to a finishing pot containing tin at 530-545° F. and a superimposed layer of oil at 460-490° F. and preferably at 470° F. The relatively high temperature was necessary to maintain the desired oil temperature. Here the sheets were immersed in the tin and then drained in the oil layer. Metal strips tested were given a tinning and oil treatment at regular intervals and the test was conducted for a period of 72 hours. The properties as indicated in Table I were graded in descending order, (1) being the best, (2) next best, etc. The results of the test were as follows:

kept at a temperature of 460-475° F. To simulate the oil-tin interface encountered in tinplate manufacture, a small amount of tin was poured into the bottom of the oil pot. Tests were conducted for a 72 hour period with the same compositions as indicated in Table I and the results were substantially the same as indicated in Table I.

C. Still another test was conducted in a small 10 tinning machine similar to that described in columns 1 and 2. The tin was melted, put in the oil pot and the flux and oil tested put in the feed and end or exit compartments of the machine respectively. The oil temperature was kept in the range of 475-490° F. Approximately three 15 tests with each oil were conducted during a 24 hour interval and the tinning performance of the oils as to flux removal, draining characteristics, ease of cleaning and spreading characteristics were noted. The results again were similar to those disclosed in Table I, showing the su- 20

TABLE I

[The rating as here given is an arbitrary figure which is based on the figure 1 as being excellent and 10 as being unsuitable for tin coating and the like.]

| Code No.                        | Flux Removal                                  | Draining Characteristics                                                       | Ease of Cleaning                                              | Spreading Characteristics                         | Total | Remarks                                                                                                                                                                                                                                                                               |
|---------------------------------|-----------------------------------------------|--------------------------------------------------------------------------------|---------------------------------------------------------------|---------------------------------------------------|-------|---------------------------------------------------------------------------------------------------------------------------------------------------------------------------------------------------------------------------------------------------------------------------------------|
| 1.....                          | 10. Poor flux removal.                        | 10. Streaked badly.                                                            | 10. Flux spots, Stained, sticky and difficult to clean.       | 10. Stained, Stripped, Heavy tin-need.            | 40    | Mineral alone was found totally unsuitable. At the end of 24 hours sludge formations were high and losses heavy so that test had to be discontinued.                                                                                                                                  |
| 2.....                          | 3. Showed good flux removal for 72 hour test. | 5. Good draining characteristics for early part of.                            | 4. Easy but flux spots noted.                                 | 3. Good at early stage but spangled about 24 hrs. | 15    | Although the tinning characteristics of palm oil were good for 24 hours, oil losses were heavy at the end of the 72 hour test.                                                                                                                                                        |
| 3. 30% Palm oil in mineral oil. | 6.....                                        | 8. Poor throughout test period.                                                | 8. Easy to remove but flux spots noted.                       | 7. Stained.....                                   | 29    | After 24 hours the tin plate was stained and spangled. Stripping was noted and draining was poor throughout test. At the end of 24 hours test was discontinued.                                                                                                                       |
| 4.....                          | 3.....                                        | do.....                                                                        | 8. Good draining early period of test but became worse later. | 4. Fair.....                                      | 21    | Flux removal and spreading were good. Draining and cleaning were poor and became increasingly worse.                                                                                                                                                                                  |
| 5.....                          | 2. Good.....                                  | 3. Good for 48 hours, but at end of test period showed signs of poor draining. | 3. Same.....                                                  | 2. Good.....                                      | 10    | Flux removal and spreading were good. Exhibited a pronounced stabilizing effect on the composition and gave good tinning performance at the end of 48 hours and fair tinning performance at the end of 72 hours. Oil losses were only $\frac{1}{3}$ of that of palm oil after 72 hrs. |

Code No. 1—Mineral oil (Solvent extracted Mid-Continent oil (150-170 SUS at 210° F.)).

Code No. 2—Palm oil.

Code No. 3—20-50% by wt. of palm oil in mineral oil base.

Code No. 4—Mixture of hydrogenated fish oil residuum or stearine pitches in mineral oil having an acid number of 3 to 15.

Code No. 5—Mixture of hydrogenated fish oil distillates in mineral oil having an acid value of 3 to 15.

B. Another test was conducted in which the tinning technic was slightly modified. Two tinning pots were used as before, and the temperature of the first tin pot was kept at 535° F. and the final pot at 475° F. Instead of the oil layer on the second pot, a small amount of tallow just sufficient to form a ring covering the bath edges was used to keep the surface clean. Im-

poriety of mineral oil-hydrogenated fish oil distillates over other oils tested as tinning oil.

D. Tests were conducted according to procedure outlined under A and B in order to determine the criticality of maintaining the acid number of mineral oil-hydrogenated fish oil distillates between about 3 to 15. The following results were obtained.

TABLE II  
Comparative rating as to the following characteristics.<sup>1</sup>

|   | Agent                                                                                   | Flux Removal | Draining Characteristics | Ease of Cleaning | Spreading Characteristics | Total | Remarks                                                |
|---|-----------------------------------------------------------------------------------------|--------------|--------------------------|------------------|---------------------------|-------|--------------------------------------------------------|
| 1 | Mineral oil-hydrogenated fish oil distillates having an acid number less than 3.        | 8            | 9                        | 7                | 6                         | 30    | Drained very poorly and unstable.                      |
| 2 | Mineral oil-hydrogenated fish oil distillates having an acid number greater than 15.    | 3            | 6                        | 7                | 4                         | 20    | Cause etching of metal surface and difficult to clean. |
| 3 | Mineral oil-hydrogenated fish oil distillates having an acid number between about 4-10. | 2            | 3                        | 3                | 2                         | 10    | Good spreading characteristics and stable.             |

<sup>1</sup> The rating as here given is an arbitrary figure which is based on the figure 1 as being excellent and 10 as being unsuitable for tin coating and the like.

mediately upon withdrawal of the sheet from the second pot, it was transferred to an oil pot

As has been repeatedly pointed out the acid number of tinning oil composition of this in-

vention must be kept at not less than 3 and not over 15. Since compositions of this invention are modified due to the elevated temperature at which they are maintained, readjustment of the acid value within the desired limit must be made at certain intervals. This is done by replenishing the composition with a concentrate comprising approximately 50% by weight mineral oil and 50% by weight partially hydrogenated fish oil distillates in amount sufficient to maintain the acid number of the composition between about 3 to 15, and preferably 4 to 10. By replenishing composition of this invention with the above concentrate such tinning oils can be used with excellent results for many months.

The amount of partially hydrogenated fish and/or marine oil distillates added to a mineral oil base may vary between about 2 to 20% by weight and preferably between about 5 to 15% by weight based on the amount of mineral oil used.

A quick and conclusive test was developed to study the draining characteristics of tinned oils. A heavily tinned plate was immersed for 15 seconds into an oil kept at a temperature of approximately 480° F. Heavily tinned plates were repeatedly dipped in the various oils during a 24 hour interval and the characteristics of the oil film remaining on the plate were preserved by printing off on a hard filter paper and observations made.

TABLE III

|   | Composition                                                                           | Observations and Remarks                                                           |
|---|---------------------------------------------------------------------------------------|------------------------------------------------------------------------------------|
| 1 | Mineral Oil.....                                                                      | Drained poorly throughout test period. Filter paper covered with a heavy oil film. |
| 2 | 30% by wt. of Palm Oil in mineral oil.                                                | Drained poorly, paper covered with an oil film.                                    |
| 3 | Mineral oil-hydrogenated fish oil distillates having an acid number less than 3.      | Do.                                                                                |
| 4 | Palm Oil.....                                                                         | Drained very well, few oil spots on paper.                                         |
| 5 | Mineral oil-hydrogenated fish oil distillates having an acid number between 3 and 15. | Equal to, if not superior to, palm oil in draining characteristics.                |

Modifications as to procedure of tinning and composition can be made in order to obtain an improved tinplate with the use of composition of this invention. Thus the life of the oil can be extended and the tinning surface can be improved by carrying out the entire tinning operation in enclosed vessels and in the absence of air and other oxidizing mediums. In addition, minor amounts of high molecular fatty acids such as oleic, stearic and the like can be added to compositions of this invention to improve the lustre of the tinplate, and spreadability of the tinning composition. Also animal and vegetable oils such as cocoanut oil, castor oil, cotton-seed oil, peanut oil and the like as well as synthetic lubricants produced by polymerization of olefins can be admixed with composition of this invention.

Compositions of this invention are not restricted to use in tinplating only but are equally applicable for terne coating, lead coating and the like. Neither are these compositions restricted to use where metal plating is done only by dipping and the like. Compositions of this invention can be used to improve the metal-coating surface and deposition of metals on metal base by electrolytic methods as well as any other known metal plating method. The appearance of surfaces having tin deposited thereon by elec-

trolytic means is greatly improved by dipping such metal treated surfaces into a hot bath comprising an oil composition of this invention.

In addition to being equal to and in most properties superior to palm oil, compositions of this invention have a particular advantage over palm oil in that they reduce to a minimum the danger of fire hazard.

It is to be understood that while the features of the invention have been described and illustrated in connection with specific compositions, the invention is not to be limited thereto or otherwise restricted, except by the prior art and the scope of the appended claims.

15 I claim as my invention:

1. A method of coating ferrous metal which includes cleaning and pickling said metal, passing the metal through a flux bath consisting essentially of a zinc chloride-ammonium chloride solution, followed by passing the metal into a molten tin bath maintained at a temperature between about 530°-560° F. and finally passing said tin treated metal through an oil composition maintained at a temperature between about 460°-490° F. consisting essentially of a mixture of mineral oil and partially hydrogenated fish oil distillates, said oil mixture having an acid number of not less than 3 and not more than about 15.

2. A method of coating ferrous metal which includes cleaning and pickling said metal, passing the metal through a flux bath consisting essentially of a zinc chloride-ammonium chloride solution, followed by passing the metal into a molten tin bath maintained at a temperature between about 530°-560° F. and finally passing said tin treated metal through an oil composition, maintained at a temperature between about 460°-490° F., consisting essentially of a mixture of mineral oil and partially hydrogenated fish oil distillates, said oil mixture being replenished at desired intervals with a concentrate comprising approximately a 50-50 mixture of hydrogenated fish oil distillates-mineral oil, in amounts sufficient to maintain the acid number of said oil composition between about 3 to 15.

3. A method of coating ferrous metal which includes cleaning and pickling said metal, passing the metal through a flux bath consisting essentially of a zinc chloride-ammonium chloride solution, followed by passing the metal into a molten tin bath maintained at an elevated temperature and finally passing said tin treated metal through an oil composition, maintained at an elevated temperature, consisting essentially of a mixture of mineral oil and partially hydrogenated fish oil distillates, said oil mixture being replenished at desired intervals with a concentrate comprising approximately a 50-50 mixture of hydrogenated fish oil distillates-mineral oil, in amounts sufficient to maintain the acid number of said oil composition between about 3 to 15.

4. A method of coating ferrous metal which includes cleaning and pickling said metal, passing the metal through a flux bath, on through a molten metal bath selected from the class consisting of molten tin, tin-lead alloy and lead and finally passing said metal through an oil composition, maintained at an elevated temperature, consisting essentially of a blend of mineral oil and partially hydrogenated marine oil distillates, said oil blend having an acid number of not less than 3 and not more than about 15.

5. A method of coating ferrous metal which includes cleaning and pickling said metal, passing the metal through a flux bath, on through a

molten metal bath of tin and finally passing said metal through an oil composition, maintained at an elevated temperature, consisting essentially of a blend of mineral oil and partially hydrogenated fish oil distillates, said oil blend having an acid number of not less than 3 and not more than about 15.

6. A method of coating ferrous metal which includes cleaning and pickling said metal passing the metal through a flux bath, on through a molten metal bath of tin-lead alloy and finally passing said metal through an oil composition, maintained at an elevated temperature, consisting essentially of a blend of mineral oil and partially hydrogenated fish oil distillates, said oil blend having an acid number of not less than 3 and not more than about 15.

7. A method of coating ferrous metal which includes cleaning and pickling said metal passing the metal through a flux bath, on through a molten metal bath of lead and finally passing said metal through an oil composition, maintained at an elevated temperature, consisting essentially of a blend of mineral oil and partially hydrogenated fish oil distillates, said oil blend having an acid number of not less than 3 and not more than about 15.

8. A mineral oil composition suitable for aiding the formation of an adherent metal coating on another metal, consisting essentially of a mixture of a mineral oil and a hydrogenated fatty oil distillate, said blend having an acid number of between about 3 to 15.

9. A mineral oil composition suitable for aiding in the formation of an adherent metal coating on the surface of an article of another metal, consisting essentially of a mixture of a mineral oil and a hydrogenated marine oil distillate, said blend having an acid number of between about 3 and 15.

10. A mineral oil composition suitable for aiding in the formation of an adherent metal coating on the surface of an article of another metal, consisting of a mixture of a mineral oil and a hydrogenated marine oil distillate, said blend having an acid number of between about 3 and 15.

11. A mineral oil composition suitable for aiding in the formation of an adherent metal coating on the surface of an article of another metal, consisting of a mixture of 2% to 20% of a hydrogenated marine oil distillate and the balance mineral oil.

12. A soap-free, non-emulsifiable mineral oil

composition suitable for aiding in the formation of an adherent metal coating on the surface of an article of another metal, consisting of a mixture of from 5% to 15% of a hydrogenated marine oil distillate and the balance mineral oil.

13. A mineral oil composition suitable for aiding in the formation of an adherent metal coating on the surface of an article of another metal, consisting of a mixture of a mineral oil and a hydrogenated fish oil distillate, said blend having an acid number of between 3 and 15.

14. A mineral oil composition suitable for aiding in the formation of an adherent metal coating on the surface of an article of another metal, consisting of a mixture of 2% to 20% of a hydrogenated fish oil distillate and the balance mineral oil.

15. A soap-free, non-emulsifiable mineral oil composition suitable for aiding in the formation of an adherent metal coating on the surface of an article of another metal, consisting of a mixture of from 5% to 15% of a hydrogenated fish oil distillate and the balance mineral oil.

16. A mineral oil composition suitable for aiding in the formation of an adherent metal coating on the surface of an article of another metal, consisting of a mixture of 2% to 20% of a hydrogenated fatty oil distillate and the balance mineral oil.

17. A method of coating ferrous metal which includes cleaning and pickling said metal, passing the metal through a flux bath on through a molten metal bath selected from the group consisting of tin, tin-lead alloy and lead and finally passing said metal through an oil composition, maintained at an elevated temperature, consisting essentially of a mineral oil and a hydrogenated fatty oil distillate, said oil blend having an acid number of not less than 3 and not more than about 15.

40 GEORGE W. WATERS.

#### REFERENCES CITED

The following references are of record in the file of this patent:

#### UNITED STATES PATENTS

| Number       | Name                   | Date          |
|--------------|------------------------|---------------|
| 1,998,767    | MacLaren et al. _____  | Apr. 23, 1935 |
| 50 2,044,210 | Gordon _____           | June 16, 1936 |
| 2,229,368    | Brunstrom et al. _____ | Jan. 21, 1941 |
| 2,291,460    | Francis _____          | July 28, 1942 |
| 2,356,863    | MacLaren et al. _____  | Aug. 29, 1944 |